

March 20, 1934.

W. S. KELLAR

1,951,874

METHOD OF MAKING VIBRATORY DEVICES

Filed Jan. 13, 1931



Inventor  
W. S. Kellar

By J. H. B. Whitefield, Atty.

## UNITED STATES PATENT OFFICE

1,951,874

## METHOD OF MAKING VIBRATORY DEVICES

William S. Kellar, Lombard, Ill., assignor to  
Western Electric Company, Incorporated, New  
York, N. Y., a corporation of New York

Application January 13, 1931, Serial No. 508,484

3 Claims. (Cl. 29—169.5)

This invention relates to vibratory devices and methods of producing the same, and more particularly to diaphragms and other vibratory devices formed of aluminum alloys, and to methods 5 of producing such devices.

The object of the invention is to provide an improved and efficient method of producing metallic vibratory devices.

The invention is particularly applicable to the 10 production of diaphragms and other vibratory parts used in the transmission, recording, and reproduction of sound, an example of such parts being a transmitter diaphragm for use in telephonic communication systems. Such diaphragms must possess the qualities of lightness, 15 strength, and elasticity, and it is an object of the present invention to produce parts which will meet these as well as other requirements.

In one embodiment, wherein the invention is 20 applied to the production of telephone transmitter diaphragms, the metal from which the diaphragms are to be made consists of an aluminum alloy which is formed into a strip and annealed at a temperature sufficiently low to avoid dis- 25 coloring the metal. The annealed strip is then reduced to the thickness desired in the finished diaphragms and the diaphragms are then blanked from the strip. The blanks are then heat-treated at a higher temperature and are shaped, by 30 stamping or otherwise, into their final form im- mediately after the heat-treatment. The dia- phragms are then age hardened for several days after which they are ready to be assembled into telephone transmitters.

The invention will be more fully understood 35 from the following description taken in connection with the appended drawing, in which the single figure is a fragmentary sectional view of a telephone transmitter comprising a diaphragm 40 which may be formed in accordance with the invention.

The preferred composition of the alloy from 45 which the vibrating parts are made is as follows:

|                |                    |
|----------------|--------------------|
| Copper-----    | 3.15% to 4.50%     |
| Silicon-----   | .20% to .50%       |
| Magnesium----- | .40% to 1.00%      |
| Manganese----- | .40% to 1.00%      |
| Iron-----      | Not more than .50% |
| Aluminum-----  | Balance            |

The alloy is first reduced to the form of a strip about  $2\frac{1}{8}$ " wide and .020" thick and the strip is annealed at a temperature below that which will cause discoloration or oxidization, a temperature 55 of about 660° to 700° F. being preferred. It is

then cooled in air and reduced by cold-rolling to its final thickness, which may be .003" or thereabouts. The diaphragm blanks or disks are then formed from the strip by punching or otherwise, and these blanks are then heat-treated by main- 60 taining them at a temperature of from 930° to 960° F. for about seven minutes. To avoid dis- coloring, it is desirable to bring all the blanks up to temperature quickly and simultaneously without overheating any of them, hence the 65 blanks should be scattered or arranged in such a way as to expose all their surfaces to the heat of the furnace, rather than to mass or stack them in regular formation, and only a limited number of blanks should be introduced into the furnace 70 at one time, so that they may be raised to the desired temperature within about two minutes. After being maintained at a temperature of 930° to 960° F. for about seven minutes, the blanks are formed by stamping into the shape shown in 75 the drawing, wherein one face of the diaphragm 8 is concave and the other convex, and corruga- tions 10 extend radially of the diaphragm.

This forming operation should be performed 80 within a limited time, preferably one hour, after the disks are heat-treated, and this may necessitate heat-treating at one time only a limited number of disks corresponding to the number of disks which can be stamped into final form 85 within one hour. The necessity for forming the disks quickly after heat-treatment arises from the fact that the alloy age hardens after the heat-treatment and at the end of about one hour has hardened to such an extent that forming it would produce undesirable internal stresses which 90 would tend to produce cracks or flaws in the finished diaphragms.

The diaphragms after being formed are age hardened by maintaining them at room tempera- 95 ture for about four days, after which they are ready to be assembled into a telephone trans- mitter such as is shown in the drawing. The material in the finished diaphragm has a tensile strength of about 55,000 pounds per square inch.

The invention is also capable of use in con- 100 nection with the production of diaphragms or membranes designed to respond to pressure fluctuations in pressure reducing valves and similar apparatus where lightness, strength, and sensitivity to variations in pressure are desired. Such 105 diaphragms or membranes are not usually free to vibrate in the same manner as is the dia- phragm above described, but are designed to be moved out of a normal position by exterior forces and to be restored to such normal position by 110

the elasticity of the material, and are therefore intended to be included within the term "vibratory devices" as it is used in this application. The term "aluminum base alloy" is used in the following claims to designate an alloy of the kind described in the above description.

The invention is also capable of other modifications and embodiments, and its scope is not limited except by the terms of the following claims.

10 What is claimed is:

1. The method of producing a vibratory device having an irregular cross-section, which comprises reducing to a form having a plane cross-section an aluminum alloy having substantially

15 the following composition: 3.15% to 4.50% copper, .20% to .50% silicon, .40% to 1.00% magnesium, .40% to 1.00% manganese, balance aluminum, heat-treating the alloy at from 930° to

20 960° F. for about seven minutes, and forming

the alloy into a form having an irregular cross-section within three hours after the heat-treatment.

2. The method of producing a vibratory device which comprises reducing an aluminum base alloy comprising substantially 4% copper, substantially 90% aluminum, and small amounts of silicon, magnesium, manganese and iron to sheet form, heating the sheet to the vicinity of 660° to 700° F., cooling the sheet in air, cold working the sheet, heating the sheet to the vicinity of 930° to 960° F. for approximately seven minutes, and forming the sheet into a vibratory device 85 within a short time after the last heat-treatment.

3. The method of producing a vibratory device which comprises reducing an aluminum base alloy to sheet form, heating the sheet to the vicinity of 660° to 700° F., cold working the sheet, heating the sheet to the vicinity of 930° to 960° F. for about seven minutes, and forming the sheet into a vibratory device within a short time after the last heat-treatment. 90 95

WILLIAM S. KELLAR.

25

100

30

105

35

110

40

115

45

120

50

125

55

130

60

135

65

140

70

145

75

150